

Aug. 13, 1929.

J. MacLAURIN

1,724,672

ORNAMENTAL PAPER AND METHOD OF MANUFACTURING SAME

Filed Nov. 3, 1925

FIG. 1.



FIG. 2.

INVENTOR.  
John MacLaurin  
BY G. S. McCrea  
his ATTORNEY.

Patented Aug. 13, 1929.

1,724,672

# UNITED STATES PATENT OFFICE.

JOHN MACLAURIN, OF WARE, MASSACHUSETTS.

ORNAMENTAL PAPER AND METHOD OF MANUFACTURING SAME.

Application filed November 3, 1925. Serial No. 68,659.

This invention relates to papers, fabrics, and the like, hereinafter referred to as "paper", which are coated or otherwise treated to produce ornamental effects.

5 The invention provides a unique article of this character, and it also involves a thoroughly practical method of manufacturing such an article.

I have found that very unusual and pleasing effects can be produced by coating paper, or the like, with certain substances which, upon drying, produce flake-like crystals. Especially pleasing effects are produced by coating paper with a solution of manna or 10 mannitol and then so controlling the drying of the solution on the paper that large flake-like crystals will form, the crystals spreading until they meet each other. These crystals are iridescent and if the solution 15 is colored or tinted, very attractive and unique results are produced. For example, the solution may be so colored that the crystals will have a delicate pink tint, in which case they resemble shell pearl formations 20 and unitedly they form a coating of unusual beauty.

Commercial manna of either the small flake or large flake variety may be used successfully, but I prefer to extract it by dissolving the commercial product in boiling water, allowing it to cool, and then filtering off the crystals. This removes many of the impurities, produces a material having a better color, and removes the tacky constituent 25 of the original manna, leaving essentially a material which is known as mannitol or mannite, although this material may perhaps still be associated with some impurities. I have produced very satisfactory results by dissolving fifty pounds of mannitol, or manna after being extracted as 30 above described, in fifty pounds of water, and adding to this solution four ounces of gum tragacanth, two ounces of glycerine, and the desired coloring matter to tint the 35 solution. This solution is applied to the paper, or the like, while hot, say at a temperature of 175° F., and the paper so coated is then allowed to dry. It appears to be 40 very important for the production of the large flake-like crystals which are desired to avoid disturbing the coating after it has once been applied to the paper and also to 45 control or regulate the rate of drying of the coating so that it will not proceed too rapidly.

In the drawings—

Figure 1 is a diagrammatic view showing an apparatus with which the present process may conveniently be practiced; and

Fig. 2 is a plan view of a portion of a sheet of paper coated in accordance with this invention.

Referring to Fig. 1 it will be seen that the paper to be coated is unwound from the supply roll 2 and is led over guide rolls 3 and 4 to a dip roll 5 which is partly submerged in the coating solution held in the tank 6. The solution is maintained at the desired temperature by heat supplied from any convenient source, as for example, from a gas burner 7, although a water jacketed tank is preferable to one directly heated. The paper passes between the roll 5 and a squeeze roll 8, is led out of the tank and over guide rolls which engage the uncoated surface of the paper, and it then goes to a suitable festooning mechanism. The thickness of the coating applied is determined by the adjustment of the distance between the squeeze roll 8 and the roll 5, and it is preferable, also, to maintain the level of the coating solution in the tank 6 substantially at the height of the bite of the rolls 5 and 8. It will be observed that this arrangement leaves the coated surfaces of the paper undisturbed after it comes from the coating bath, and this appears to be essential to the proper formation of the crystals desired.

The rate of drying of the coating may be controlled by properly regulating the humidity in the room where the coating operation is carried on. It is more economical and generally preferable, however, to accomplish this result through the use of a hygroscopic agent in the coating compound, and preferably a hygroscopic adhesive agent is used for this purpose, the adhesive producing a firmer bond between the mannitol crystals and the paper. It is for this purpose that the gum tragacanth and glycerine are used in the formula above given since these materials combined form an adhesive having a high affinity for water. The gum tragacanth may, however, be replaced by starch, Irish moss, or other suitable adhesives. If the adhesives used has sufficient affinity for water, the glycerine may be omitted.

The rate of drying of the coating should be so controlled that in from five to fifteen minutes after the coated paper has left the

5 tank, small crystals begin to appear, first showing simply as points, and gradually growing or spreading until they meet, so that the entire coating finally consists of 5 flat flake-like crystals, irregular in shape, and lying edge to edge. The crystals grow or spread gradually so that the coating may not be crystallized for its entire width until perhaps thirty minutes after it has left the 10 tank. It is very difficult to illustrate in a drawing the product resulting from this method, but applicant has endeavored to show the coated paper in Fig. 2, the points at which the crystals start being shown at 9.

15 As soon as the crystals have completely formed, the drying operation may then be hastened artificially as by running the paper over a drying drum, the temperature of which is properly regulated, and the coated 20 web may then be wound up in the usual manner.

As above stated, this process produces very unusual and pleasing results. The crystalline coating has a soft satiny appearance 25 which is very attractive indeed, particularly when the color used in the coating solution is appropriately chosen. Such papers are especially adapted for box coverings, envelope linings, and a great variety of other uses.

30 While I have herein disclosed a formula which has produced very satisfactory results, it will be understood that this disclosure is made rather by way of illustration than 35 limitation, and that not only may a great variety of formulae be used but that the process of the invention may be practiced in different ways and with many different forms of apparatus.

40 Having thus described my invention, what I desire to claim as new is:

1. An article of the character described comprising a sheet of paper having thereon an ornamental coating of flake-like crystals 45 comprising mannitol associated with a small percentage of a hygroscopic agent.

2. An article of the character described comprising a sheet of paper having thereon an ornamental coating of flake-like crystals 50 joined edge to edge, said crystals consisting chiefly of mannitol associated with a small percentage of a hygroscopic adhesive agent.

3. An article of the character described comprising a sheet of paper having thereon an ornamental coating of flake-like crystals 55 joined edge to edge, said crystals consisting essentially of mannitol associated with small percentages of coloring material and hygroscopic adhesive agent.

4. That improvement in the process of 60 manufacturing ornamental paper which consists in coating a sheet of paper with a coating compound consisting chiefly of a solution of mannitol, drying the paper so coated, and so controlling the rate of drying of the 65 coating that flake-like crystals will form on said paper with the edges of said crystals substantially meeting each other.

5. That improvement in the process of 70 manufacturing ornamental paper which consists in coating a sheet of paper with a coating compound consisting chiefly of a solution of mannitol, drying the paper so coated, leaving the coating undisturbed while it 75 dries, and so regulating the rate of drying that flat flake-like crystals will form in the coating and spread until they substantially meet each other.

6. That improvement in the process of 80 manufacturing ornamental paper which consists in coating the paper with a solution of mannitol, allowing the paper so coated to dry, and using a hygroscopic agent in said solution to control the rate of drying of the 85 coating so that the greater part of said coating will be converted into flake-like crystals.

7. That improvement in the process of 90 manufacturing ornamental paper which consists in coating paper with a hot aqueous solution of mannitol associated with a coloring material and a small percentage of a hygroscopic adhesive substance, leaving the 95 coated surface undisturbed while it dries, and so regulating the rate of drying that flat flake-like crystals will form in the coating during drying and spread until they substantially meet each other.

8. An article of the character described comprising a sheet of paper, having thereon an ornamental coating of flake-like crystals 100 consisting essentially of mannitol associated with a small percentage of an adhesive agent.

JOHN MACLAURIN.